

## UNITED STATES PATENT OFFICE

2,597,856

## STABILIZATION OF PHOTOGRAPHIC EMULSIONS SENSITIZED WITH GOLD COMPOUNDS

Rudolph E. Damschroder, Rochester, N. Y., assignor to Eastman Kodak Company, Rochester, N. Y., a corporation of New Jersey

No Drawing. Application September 24, 1949,  
Serial No. 117,719

20 Claims. (Cl. 95—7)

1

This invention relates to stabilization of photographic emulsions which are sensitized with gold compounds.

It is known that photographic silver halide emulsions can be sensitized by digesting the emulsions in the presence of gold compounds. The gains in speed thus obtained are clearly of value, but it has been found that coatings of such emulsions on the usual supports tend to lose speed on keeping or storage.

I have now found that the speed stability of coatings of emulsions sensitized with gold compounds can be markedly improved by the addition of at least one water-soluble gold compound to the gold-compound-sensitized emulsions after the final digestion of the emulsions but before coating the emulsions on a support. The addition of the water-soluble gold compounds after final digestion, but before coating does not increase the initial speed of the emulsion, but rather stabilizes the already sensitized emulsions against speed loss on keeping or storage of the coated emulsions.

It is, accordingly, an object of my invention to provide photographic emulsions sensitized with gold compounds, which emulsions have improved resistance to loss of speed, i. e. sensitivity, on keeping or storage. A further object is to provide a process for preparing such improved emulsions. Other objects will become apparent hereinafter.

The usual procedure for preparing photographic silver halide developing-out emulsions, especially photographic gelatino-silver-halide developing-out emulsions, comprises the following steps:

- (1) *Precipitation*.—Wherein the silver halide is precipitated by the interaction of a water-soluble silver salt and a water-soluble halide, in the presence of a carrier, e. g. gelatin.
- (2) *Digestion*.—Wherein the above precipitate is heated for a period of time at a raised temperature, e. g. 50° to 60° C., with or without the addition of further carrier, e. g. gelatin.
- (3) *Washing*.—Wherein the digested, solidified or set (e. g. by chilling) emulsion is washed to remove soluble salts.
- (4) *Melting out and second digestion*.—Wherein the washed emulsion is melted and the resulting flowable emulsion is heated for a period of time, with or without the addition of further carrier, e. g. gelatin.

Of course, variations of the above four steps can be employed. An emulsion, when used without

5 employing a step, such as (3), I call an unwashed, finished emulsion. An emulsion when used following completion of all four steps, I call a washed, finished emulsion. The latter is the type of emulsion generally used.

10 During the last step, i. e. the melting-out and second or final digestion, the emulsion increases in sensitivity. To increase the speed of photographic emulsions various substances have been added at various stages in the preparation of the emulsions. Usually the additions are made during one of the digestion periods. Frequently sulfur compounds, i. e. so-called "sulfur sensitizers" have been added, e. g. allyl isothiocyanate, thiourea, thiocarbanilide, etc., have been added. 15 More recently, it has been proposed to employ ammonium and/or metal thiocyanates for this purpose. Still more recently gold compounds have been proposed for the same purpose. It is 20 with these photographic silver halide emulsions which during their preparation have been sensitized by digestion in the presence of gold compounds with or without the additional presence of a sulfur sensitizer, that my invention is concerned.

25 In accordance with my invention, I incorporate in a photographic silver halide emulsion (which during its preparation has been sensitized by digestion in the presence of a gold compound) at least one water-soluble gold compound which has a solubility in water greater than the equivalent of 1.0 mg. of gold (metallic) per 100 ml. of water at 25° C., after the final digestion of the emulsion and before coating the emulsion on a support.

30 Typical of the water-soluble gold compounds are:

- I. Potassium chloroaurate,  $KAuCl_4$
- II. Auric trichloride,  $AuCl_3$
- III. Myochrysine (gold sodium-thiomalate)
- 40 IV. Potassium aurithiocyanate,  $KAu(CNS)_4$
- V. Solganal-B oleosum (aurothioglucose in sesame oil)
- VI. Pyridino-trichlorogold,  $(C_5H_5N)AuCl_3 \cdot HCl$
- VII. Trichlorogold-dimethyl sulfide,

45  $AuCl_3 \cdot (CH_3)_2S$

VIII.



50

IX. Diethyl-monobrom-gold,  $Au(C_2H_5)_2Br$

## X. Monochlorogold-dimethyl sulfide,

XI. Potassium aurothiocyanate,  $\text{KAu}(\text{CNS})_2$ 

The water soluble gold compounds can be added to the emulsions in the form of solutions in suitable solvents, e. g. water, methyl alcohol, ethyl alcohol, acetone, etc., or as dispersions in colloids, such as gelatin, polyvinyl alcohol, partially hydrolyzed cellulose acetate, casein, etc., or without any solvent or colloid. The water soluble gold compounds should, of course, be thoroughly dispersed throughout the emulsions, e. g. by stirring.

Ordinarily, it is advantageous to employ a concentration of the water-soluble gold compound equivalent to from 1.5 to 20 mg. of metallic gold per 1000 g. of silver nitrate used in preparing the emulsion. However, lower or greater concentrations can be employed, e. g. a concentration equivalent to 1000 mg. of metallic gold per 1000 g. of silver nitrate used in preparing the emulsion.

The water-soluble gold compounds are advantageously added to the emulsions after the final digestion, but prior to coating the emulsions on a support, at a pH of from 5 to 9, and most advantageously at pH of from 6 to 7.

The following examples will serve to illustrate further the manner of practicing my invention.

## EXAMPLE 1

A batch of gelatino-silver-bromoidide emulsion was prepared as described by Trivelli and Smith—Phot. J. 79, 330 (1939), using a precipitation time of about 20 minutes (emulsion No. 11, page 330), except that just before the final digestion of the emulsion, potassium chloroaurate ( $\text{KAuCl}_4$ ) in a concentration equivalent to 6.5 mg. of metallic gold per 1000 g. of silver nitrate employed in preparing the emulsion, thiosinamine in a concentration of 50 mg. per 1000 g. of silver nitrate employed in preparing the emulsion, and sodium thiocyanate in a concentration of 1 g. per 1000 g. of silver nitrate employed in preparing the emulsion, were added to the emulsion. A portion of the emulsion was coated on a cellulose acetate film and dried. The film was cut into two portions. One portion was kept no longer than for the short time (few hours) at about 70° F. required for the routine of exposing the film in a 1b sensitometer at  $1/25$  second exposure, using 100 watt, sunlight quality illumination and developing the exposed film in Eastman Kodak Company's "D-19" developer for 4 minutes at 20° C. The results of this exposure and development are given in Table A below. The other portion was subjected to an accelerated keeping or incubation treatment wherein the coated film was stored or kept for 7 days at 120° F. At the end of this period, the incubated film was exposed and developed as described above. Results are recorded in Table A below.

To further portions of the same emulsion after final digestion and before coating the portions of emulsion on cellulose acetate films various water-soluble gold compounds were added as shown in Table A below. The coated films were cut into two portions and one portion exposed and developed in the routine manner described above. The other portion was subjected to an accelerated keeping or incubation treatment wherein the coated film was stored or kept for 7 days at 120° F. At the end of this period, the incubated film was exposed and developed as described above. Results are recorded in Table A below.

4  
Table A

|             | Water-soluble Gold Compound After Final Digestion (mg. of gold per 1000 g. of $\text{AgNO}_3$ ) | Keeping Treatment | Speed (1/l) | Gamma | Fog |
|-------------|-------------------------------------------------------------------------------------------------|-------------------|-------------|-------|-----|
| 5           |                                                                                                 |                   |             |       |     |
| 1. none     | routine                                                                                         | 80                | 0.90        | 0.05  |     |
|             | 7 days at 120° F.                                                                               | 33                | 0.73        | 0.18  |     |
| 2. I, 2.5   | routine                                                                                         | 71                | 0.91        | 0.05  |     |
|             | 7 days at 120° F.                                                                               | 37                | 0.82        | 0.17  |     |
| 3. I, 7.5   | routine                                                                                         | 69                | 1.04        | 0.07  |     |
|             | 7 days at 120° F.                                                                               | 80                | 0.80        | 0.22  |     |
| 4. I, 20    | routine                                                                                         | 73                | 1.05        | 0.10  |     |
|             | 7 days at 120° F.                                                                               | 108               | 0.87        | 0.25  |     |
| 5. I, 50    | routine                                                                                         | 68                | 1.05        | 0.10  |     |
|             | 7 days at 120° F.                                                                               | 69                | 0.70        | 0.33  |     |
| 15          |                                                                                                 |                   |             |       |     |
| 6. II, 2.5  | routine                                                                                         | 82                | 0.87        | 0.05  |     |
|             | 7 days at 120° F.                                                                               | 35                | 0.83        | 0.21  |     |
| 7. II, 7.5  | routine                                                                                         | 69                | 0.98        | 0.06  |     |
|             | 7 days at 120° F.                                                                               | 49                | 0.91        | 0.22  |     |
| 8. II, 20   | routine                                                                                         | 71                | 1.02        | 0.09  |     |
|             | 7 days at 120° F.                                                                               | 82                | 0.88        | 0.25  |     |
| 9. III, 5   | routine                                                                                         | 78                | 0.93        | 0.04  |     |
|             | 7 days at 120° F.                                                                               | 30                | 0.94        | 0.21  |     |
| 20          |                                                                                                 |                   |             |       |     |
| 10. III, 15 | routine                                                                                         | 69                | 0.96        | 0.07  |     |
|             | 7 days at 120° F.                                                                               | 68                | 0.79        | 0.22  |     |
| 11. III, 40 | routine                                                                                         | 78                | 1.02        | 0.06  |     |
|             | 7 days at 120° F.                                                                               | 94                | 0.92        | 0.23  |     |
| 12. IV, 2.5 | routine                                                                                         | 73                | 0.96        | 0.05  |     |
|             | 7 days at 120° F.                                                                               | 39                | 1.12        | 0.16  |     |
| 13. IV, 7.5 | routine                                                                                         | 73                | 0.95        | 0.06  |     |
|             | 7 days at 120° F.                                                                               | 44                | 1.00        | 0.18  |     |
| 25          |                                                                                                 |                   |             |       |     |
| 14. IV, 20  | routine                                                                                         | 52                | 1.14        | 0.05  |     |
|             | 7 days at 120° F.                                                                               | 78                | 0.91        | 0.11  |     |

From the data in the foregoing table, it is apparent that the emulsion which was sensitized by digesting in the presence of the gold compound, thiosinamine and sodium thiocyanate had a high initial speed of 80 as shown at 1. After subjecting this emulsion to an accelerated keeping treatment, however, the emulsion had lost a very large fraction of its speed (sensitivity) as shown at 1. On the other hand when potassium chloroaurate (I) was added to the same emulsion, in a concentration equivalent to 2.5 mg. of gold, after final digestion but before coating, the initial speed (71) of the emulsion was reduced to only 37 after the same accelerated keeping treatment, as shown at 2. When potassium chloroaurate (I) was added to the same emulsion, in a concentration equivalent to 7.5 mg. of gold, after final digestion but before coating, the initial speed of 69 was not reduced at all after the same accelerated keeping treatment as shown at 3. Actually, in this last instance, there was a gain rather than a loss in speed after the accelerated keeping treatment. It is to be understood, of course, that the accelerated keeping treatment is drastic and that such severe conditions would rarely be encountered in practical keeping or storage of products comprising sensitized emulsions. The other data given in the above table at 4 to 14 show further beneficial retardation of loss of speed that can be attained in accordance with my invention.

## 60

## EXAMPLE 2

A batch of gelatino-silver-bromoidide emulsion was prepared as described by Trivelli and Smith—Phot. J. 79, 330 (1939), using a precipitation time of about 20 minutes (emulsion No. 11, page 330), except that just before the final digestion of the emulsion potassium chloroaurate, thiosinamine and sodium thiocyanate were added to the emulsion in the concentrations shown in Example 1. A portion of the emulsion was coated on cellulose acetate film and dried. The film was cut into two portions and the one portion exposed and developed in the routine manner shown in Example 1 while the other portion was incubated and then exposed and

## 5.

developed as shown in Example 1. Results are recorded in Table B below.

To further portions of the same emulsion after final digestion and before coating the portions of emulsion on cellulose acetate films various water-soluble gold compounds were added as shown in Table B below. The coated films were cut into two portions and one portion exposed and developed in the routine manner described in Example 1. The other portions were incubated and then exposed and developed as described in Example 1. Results are recorded in Table B below.

Table B

| Water-soluble Gold Compound After Final Digestion, (mg. of gold per 1000 g. of $\text{AgNO}_3$ ) | Keeping Conditions     | Speed (1/10) | Gamma | Fog  |
|--------------------------------------------------------------------------------------------------|------------------------|--------------|-------|------|
| none.....                                                                                        | {routine.....          | 76           | 0.90  | 0.06 |
|                                                                                                  | {7 days at 120° F..... | 35           | 0.92  | 0.16 |
| V, 10.....                                                                                       | {routine.....          | 79           | 0.91  | 0.05 |
|                                                                                                  | {7 days at 120° F..... | 58           | 0.97  | 0.17 |
| V, 30.....                                                                                       | {routine.....          | 76           | 0.89  | 0.05 |
|                                                                                                  | {7 days at 120° F..... | 59           | 0.92  | 0.19 |
| V, 100.....                                                                                      | {routine.....          | 68           | 1.00  | 0.07 |
|                                                                                                  | {7 days at 120° F..... | 90           | 1.02  | 0.25 |
| VI, 5.....                                                                                       | {routine.....          | 74           | 0.92  | 0.07 |
|                                                                                                  | {7 days at 120° F..... | 63           | 0.99  | 0.16 |
| VI, 15.....                                                                                      | {routine.....          | 74           | 1.00  | 0.07 |
|                                                                                                  | {7 days at 120° F..... | 59           | 0.94  | 0.23 |
| VI, 50.....                                                                                      | {routine.....          | 68           | 1.03  | 0.11 |
|                                                                                                  | {7 days at 120° F..... | 80           | 0.85  | 0.31 |
| VII, 5.....                                                                                      | {routine.....          | 66           | 0.95  | 0.06 |
|                                                                                                  | {7 days at 120° F..... | 49           | 0.96  | 0.18 |
| VII, 15.....                                                                                     | {routine.....          | 71           | 1.00  | 0.09 |
|                                                                                                  | {7 days at 120° F..... | 62           | 0.91  | 0.24 |
| VII, 50.....                                                                                     | {routine.....          | 68           | 1.04  | 0.11 |
|                                                                                                  | {7 days at 120° F..... | 73           | 0.92  | 0.33 |
| VIII, 5.....                                                                                     | {routine.....          | 68           | 0.93  | 0.10 |
|                                                                                                  | {7 days at 120° F..... | 39           | 0.82  | 0.25 |
| VIII, 15.....                                                                                    | {routine.....          | 65           | 1.02  | 0.10 |
|                                                                                                  | {7 days at 120° F..... | 62           | 0.80  | 0.21 |
| VIII, 50.....                                                                                    | {routine.....          | 61           | 0.99  | 0.22 |
|                                                                                                  | {7 days at 120° F..... | 47           | 0.78  | 0.38 |
| XI, 2.5.....                                                                                     | {routine.....          | 56           | 1.01  | 0.04 |
|                                                                                                  | {7 days at 120° F..... | 45           | 0.75  | 0.18 |
| XI, 7.5.....                                                                                     | {routine.....          | 45           | 0.99  | 0.02 |
|                                                                                                  | {7 days at 120° F..... | 46           | 0.75  | 0.19 |

As in Table A, the above data in Table B show further the beneficial retardation of loss of speed that can be attained in accordance with my invention.

Any gold compound having a solubility in water greater than the equivalent of 1.0 mg. of gold per 100-ml. of water at 25° C. and be employed to add to the gold-compound-sensitized emulsions after final digestion but prior to coating of the emulsion, in accordance with my invention. Many of such water-soluble gold compounds are described in the chemical literature. For example, monochlorogold-dimethylsulfide is described by Ray and Sen—J. Indian Chem. Soc. 7, 72 (1930). Diethyl-monobrom-gold is described by Pope and Gibson—J. Chem. Soc. 91, 2061-2063 (1907). Trichlorogold-dimethylsulfide is described by Ray and Sen—J. Indian Chem. Soc. 7, 72 (1930). Pyridino-trichlorogold is described by Gmelin-Kraut—Handbuch der Anorg. Chem., V2, p. 292-34b<sub>2</sub>. Pyridinotrichloro-gold and still other of the water-soluble gold compounds can be prepared as shown in the following examples.

## EXAMPLE 3



A solution containing 1 g. of gold chloride in 95% ethyl alcohol was added to a solution containing 0.79 g. of pyridine in 10 cc. of 95% ethyl alcohol. A cream solid separated at once. The reaction mixture was stood for several hours at

## 6.

about 20° C. and then chilled to 0° C. The solid was collected on a filter and washed with acetone. The yield of cream crystals was 79% crude and 20% after two recrystallizations from acetone.

## EXAMPLE 4



- 15 A solution containing 1 g. of gold chloride ( $\text{AuCl}_3$ ) in 10 cc. of absolute ethyl alcohol was added to a suspension of 0.93 g. of 3,3'-dimethylthia carbocyanine chloride in 20 cc. of absolute ethyl alcohol. A brown solid separated at once. After chilling for 30 minutes at 0° C., the solid was 20 collected on a filter and washed with absolute ethyl alcohol. The yield of the gold compound formulated above was 83% crude and 59% after one recrystallization from nitromethane. The dark blue needles gave a bluish-red solution in 25 acetone.

In a manner similar to that illustrated in the foregoing Example 4 other water soluble gold compounds can be prepared from cyanine dyes. However, a great many of the gold compounds thus prepared from cyanine dyes are water insoluble, i. e. they have a solubility in water less than the equivalent of 1.0 mg. of gold per 100 ml. of water at 25° C.

Alkali metal chloroaurates, e. g. potassium and sodium chloroaurates, are well known substances, as is auric trichloride and alkali metal aurithiocyanates and alkali metal aurothiocyanates. Myochrysine is a product of Merck & Company and Solganal-B oleosum is a product of Schering Corporation.

My invention can be practiced on photographic silver halide emulsions which have been sensitized by digesting the emulsions in the presence of either water-soluble or water-insoluble gold compounds. As shown above the sensitization of emulsions by digesting with water-soluble gold compounds is well known. To so sensitize emulsions, at least one water-soluble gold compound, e. g. any of the water-soluble gold compounds set forth above, is added to the emulsion prior to or during the final digestion. Advantageously the concentration of the gold compound is equivalent to from 2.5 to 1000 mg. of gold per 1000 g. of silver nitrate used in preparing the emulsion. Most advantageously a concentration of water-soluble gold compound equivalent to from 2 to 30 mg. of gold per kilogram of silver nitrate used in preparing the emulsion is employed.

Advantageously the level of pH during the digestion of the emulsion, in the presence of the water-soluble gold compound, is maintained at or below 9, although this is not essential. Generally speaking, the best results are obtained by digesting the emulsions at a pH of from 5 to 9, in the presence of the water-soluble gold compound. Digestion of the emulsions in the presence of the gold compounds is advantageously effected at from 40° C. to 65° C., although other temperatures can be used. A temperature range of 50 to 60° C. ordinarily gives the best results.

Advantageously the emulsions sensitized by digesting with the water-soluble gold compounds are digested in the additional presence of at least one sulfur compound, e. g. a sulfur sensitizing agent, for

7

instance an organic compound containing a  
>C=S or a



group. Typical of such sulfur sensitizers are: 5



Normal gelatins contain small amounts of sulfur compounds, such as thiosinamine or allylisothiocyanate, but it is nevertheless frequently advantageous to add to the gelatin emulsions additional sulfur sensitizers.

Beneficial effects are also obtained by digesting the emulsions which are sensitized by digestion in the presence of a water-soluble gold compound, in the additional presence of at least one metal or ammonium thiocyanate, e. g. alkali metal thiocyanates (e. g. sodium or potassium thiocyanate), alkaline earth metal thiocyanates (e. g. calcium, strontium thiocyanate, etc.), cadmium thiocyanate, ammonium thiocyanate, etc. Of course, thiocyanates containing cations which cations are known to have, in themselves, a deleterious effect on silver halide emulsions should be avoided. Otherwise, the beneficial effects attained with the thiocyanates would be partially nullified by the deleterious action of the cation. Thus iron thiocyanate which contains the iron cation should be avoided. One or more sulfur sensitizers or one or more thiocyanates selected from the group consisting of metal or ammonium thiocyanates can be employed. One or more sulfur sensitizers can be employed in conjunction with one or more thiocyanates containing a cation selected from the group consisting of metal and ammonium cations. The sulfur sensitizers and thiocyanates are advantageously incorporated in the emulsions in the form of their solutions in a suitable solvent, such as water, methyl or ethyl alcohol.

The sulfur sensitizers can be incorporated in the emulsions at any stage of the preparation of the emulsions, e. g. during precipitation of the silver halides, during the first digestions (ripening) or during the second digestion of the emulsions. When incorporating metal and ammonium thiocyanates in the emulsions prior to washing, the amount can vary widely. Advantageously, however, an amount of thiocyanate equal to from about 10 to about 75 g. per kilogram of silver nitrate used in preparing the emulsion is employed. If the thiocyanate or sulfur sensitizer is not added until later in the preparation, e. g. after washing, it is advantageous to employ, in the case of the thiocyanates, an amount equal to from about 0.1 to about 10 g. per kilogram of silver nitrate used in preparing the emulsion and in the case of the other sulfur

8

sensitizers, an amount equal to from about 0.01 to about 10 g. per kilogram of the silver nitrate used in preparing the emulsion.

It is advantageous to digest, i. e. to heat treat, the emulsion with both the water-insoluble gold compound and the sulfur sensitizer or thiocyanate present, at an appropriate temperature, e. g. at from 100 to 150° F. During digestion, i. e. the second digestion as contrasted with the first digestion or ripening, the pH of the emulsion is advantageously adjusted to between 5 and 7.

Typical water-insoluble gold compounds with which photographic silver halide emulsions can be sensitized by digesting the emulsions in the presence thereof are described in the following examples. To sensitize emulsions with these water-insoluble gold compounds, the procedures (e. g. pH, temperature, sulfur sensitizers, thiocyanates, etc.) set forth above for sensitizing emulsions with water-soluble gold compounds can be employed.

**EXAMPLE 5**



A solution containing 0.33 g. of auric chloride in 10 cc. of 95% ethyl alcohol was added to 100 cc. of 95% ethyl alcohol containing 0.85 g. of 3-ethyl-2-(3)-thiothiazolo[4,5-*b*] quinolinone (prepared by heating 3-ethylrhodanine and *o*-amino-benzaldehyde in acetic acid solution according to Gränacher et al.—*Helv. Chim. Acta* 8, 890 (1925)). The above-formulated compound precipitated and after the reaction mixture stood for several hours at 20° C., the product was collected on a filter and washed with 95% ethyl alcohol. The yield of light cream crystals was 75% after one recrystallization from acetic acid.

**EXAMPLE 6**



55 A solution containing 0.34 g. of auric chloride in 10 cc. of 95% ethyl alcohol was added to a solution containing 1.11 g. of 3-ethyl-5[(3-ethyl-  
2(3)-benzoxazolylidene)ethylidene]rhodanine in 25 cc. of pyridine and 25 cc. of 95% ethyl alcohol. A reddish solid separated at once. The reaction  
60 mixture was stood at about 20° C. for several hours and then the solid was collected on a filter and washed with 95% ethyl alcohol. The yield of product was 63% crude and 12% after two recrystallizations from nitromethane. The reddish  
65 crystals had melting point 231-232° C. with decomposition.

**EXAMPLE 7**



9

A solution containing 0.5 g. of auric chloride in 10 cc. of 95% ethyl alcohol was added to a hot suspension of 1.61 g. of 3-ethyl-5-(3-ethyl-2(3)-benzothiazolylidene) rhodanine in 25 cc. of acetic acid. The reaction mixture was stood several hours at about 20° C. and the precipitated solid was filtered off and washed on the filter with 95% ethyl alcohol. The washed solid was extracted with 180 cc. of hot nitromethane. Upon chilling the hot extract, the crystals which formed were filtered off and recrystallized from 155 cc. of nitromethane. The yield of golden yellow crystals was almost 100%.

## EXAMPLE 8



A solution containing 1 g. of auric chloride in 10 cc. of absolute ethyl alcohol was added to a solution containing 0.66 g. of 2-methyl- $\alpha$ -naphthothiazole ethochloride in 10 cc. of absolute ethyl alcohol. A pale yellow solid separated at once. After chilling for one hour at 0° C., the solid was collected on a filter and washed with absolute ethyl alcohol. The yield of product was 92% crude and 53% after one recrystallization from nitromethane. The yellow needles gave a very pale yellow solution in acetone.

## EXAMPLE 9



A solution containing 1 g. of auric chloride in 10 cc. of absolute ethyl alcohol was added to a solution containing 0.73 g. of 2-[2-(1-piperidyl)-vinyl]benzothiazole methochloride in 10 cc. of absolute ethyl alcohol. After chilling for one hour at 0° C. the solid which separated was collected on a filter and washed with absolute ethyl alcohol. The yield was 94% crude and 67% after one recrystallization from nitromethane. The dark crystals gave a pale yellow solution in acetone.

## EXAMPLE 10



A solution containing 1 g. of auric chloride in 10 cc. of absolute ethyl alcohol was added to a solution containing 0.90 g. of 1,1'-diethyl-2,2'-cyanine chloride in 20 cc. of absolute ethyl alcohol. A reddish solid separated at once. After chilling for one hour at 0° C., the solid was collected on a filter and washed with absolute ethyl alcohol. The yield of dye was 72% crude and 45% after one recrystallization from nitromethane. The dark green crystals gave a pink solution in acetone.

10

## EXAMPLE 11



A solution containing 1 g. of auric chloride in 10 cc. of absolute ethyl alcohol was added to a suspension of 1.18 g. of 3,3'-diethyl-4,5,4',5'-di-benzothiacyanine chloride in 40 cc. of absolute ethyl alcohol. A dark solid was formed at once. After chilling for one hour at 0° C. the solid was collected on a filter and washed with absolute ethyl alcohol. The yield was 93% crude and 74% after one recrystallization from nitromethane. The blue crystals gave a yellow solution in acetone.

## EXAMPLE 12



A solution containing 1 g. of auric chloride in 10 cc. of absolute ethyl alcohol was added to a suspension of 0.92 g. of 1',3-diethylthia-2'-cyanine chloride in 20 cc. of absolute ethyl alcohol. An orange solid separated at once. After chilling for one hour at 0° C., the solid was collected on a filter and washed with absolute ethyl alcohol. The yield of dye was 89% crude and 71% after one recrystallization from nitromethane. The reddish coppery needles gave an amber solution in acetone.

## EXAMPLE 13



A solution containing 1 g. of auric chloride in 10 cc. of absolute ethyl alcohol was added to a suspension of 0.93 g. of 3,3'-diethylthiacyanine chloride in 20 cc. of absolute ethyl alcohol. A pale orange solid separated at once. After chilling for one hour at 0° C., the solid was collected on a filter and washed with absolute ethyl alcohol. The yield of dye was 56% crude and 38% after one recrystallization from nitromethane. The deep red crystals with a blue reflex gave a pale yellow solution in acetone.

In a manner similar to that shown in Examples 4 to 13, other similar organic water-insoluble gold compounds can be prepared. In the heterocyclic nuclei of the organic gold compounds set forth in Examples 4 to 13, one or more of the hydrogen atoms can be replaced by a chlorine, a bromine or an iodine atom or by an alkyl or aryl group, e. g. methyl, ethyl, phenyl, etc. Still other water-insoluble gold compounds which can be used for sensitization are: aurous sulfide described for example by J. W. Mellor—"A Comprehensive Treatise on Inorganic Chemistry," Vol. III, page 611; by E. A. Schneider—Ber. 24, 2241 (1891) and by Gmelin-Kraut—V2, page 267A<sub>(a)</sub>; Au<sub>2</sub>Se<sub>3</sub> which is described by Abegg and Auerbach—"Handbuch der Anorg. Chem." Vol. 75

II, part I, page 322 and by Gmelin-Kraut—V<sub>2</sub>, page 271 (A); and AuI which is described by Mellor, loc. cit. page 608 and by Gmelin-Kraut—V<sub>2</sub>, page 282.

Sensitizing dyes of all types can be employed to spectrally (optically) sensitize my new stabilized emulsions, e. g. erythrosin, Congo Red, any of the sensitizing cyanine dyes (monomethine, trimethine, pentamethine, heptamethine, etc.), and any of the sensitizing merocyanine dyes (see United States Patent 2,078,233, dated April 27, 1937 for example), any of the sensitizing hemicyanine dyes (see United States Patent 2,166,736, dated July 18, 1939, for example), any of the sensitizing hemioxonol dyes (see United States Patent 2,216,441, dated October 1, 1940 and United States Patent 2,165,339, dated July 11, 1939, for example), etc.

My new stabilized emulsions can be coated in the usual manner on any suitable support, such as glass, cellulose nitrate film, cellulose acetate film, polyvinyl acetal resin film, etc. to desired thickness, and then set in the usual manner. Hardening agents, setting agents and supersensitizing combinations of sensitizing dyes or a supersensitizing combination of one or more sensitizing dyes and another substance can be added to the emulsions.

Emulsions in which the carrier for the silver halide is other than gelatin and which have been sensitized by digesting in the presence of a gold compound can be stabilized in accordance with my invention. Among such non-gelatin silver halide emulsions are silver halide emulsions prepared using as the vehicle or carrier polyvinyl alcohol ("polyvinyl alcohol" is herein intended to include all water-soluble hydrolyzed polyvinyl esters containing an ester group content equivalent to from 0 to 5% by weight of polyvinyl ester); silver halide emulsions prepared using as the vehicle or carrier hydrolyzed polyvinyl acetate containing an acetate group content equivalent to from 59 to 71% by weight of polyvinyl acetate; silver halide emulsions prepared using as the vehicle or carrier polyvinyl acetals containing a large proportion of polyvinyl alcohol hydroxyl groups, e. g. polyvinyl acetaldehyde acetals containing polyvinyl acetaldehyde acetal group equivalent to at least 50% by weight of polyvinyl acetaldehyde acetal and polyvinyl alcohol hydroxyl groups equivalent to at least 15% by weight of polyvinyl alcohol, polyvinyl propionaldehyde acetals containing polyvinyl alcohol hydroxyl groups equivalent to from 45 to 60% by weight of polyvinyl alcohol, and polyvinyl butyraldehyde acetals containing polyvinyl alcohol hydroxyl groups equivalent to from 60 to 80% by weight of polyvinyl alcohol, etc. Any polyvinyl compound, especially those containing only carbon, hydrogen and oxygen atoms, or those containing carbon, hydrogen, oxygen and amine nitrogen atoms or ammonium nitrogen atoms, which is soluble in a mixture of ethyl alcohol and water (containing from 0 to 50% by volume of ethyl alcohol) to the extent of 10 g. per 100 g. of solvent can be employed as the vehicle or carrier in preparing my non-gelatin silver halide emulsions. Moreover, any other resinous or colloidal material soluble in any ethyl alcohol-water mixture or in water, as stated above, can be employed in preparing my non-gelatin silver halide emulsions, e. g. soluble polyamide resins, such as described in United States Patent 2,384,072, dated September 4, 1945, and hydrolyzed copolymers of vinyl esters and ethylene or

propylene, such as described in United States Patent 2,397,866, dated April 2, 1946. Still further examples of colloidal materials which can be employed as vehicles or carriers in preparing my non-gelatin emulsions are hydrolyzed cellulose carboxylic esters, such as hydrolyzed cellulose acetate or hydrolyzed cellulose acetate propionate, containing from 19 to 33% by weight of acyl groups, for example. Any cellulose compound, especially those containing only carbon, hydrogen and oxygen atoms, or those containing only carbon, hydrogen, oxygen and amino nitrogen atoms or ammonium nitrogen atoms, which is soluble in a mixture of ethyl alcohol and water (containing from 0 to 50% by volume of ethyl alcohol) to the extent of 10 g. per 100 g. of solvent can be employed as the vehicle or carrier in preparing my non-gelatin silver halide emulsions.

In connection with the non-gelatin colloidal materials, such as polyvinyl alcohol, the silver halide emulsions can be prepared using gelling agents, such as phenols, e. g. orcinol, gallic acid, 2,4-dihydroxybenzoic acid, 4-chlororesorcinol,  $\alpha$ -naphthol, phloroglucinol, 2,7-dihydroxynaphthalene, etc. Moreover, the non-gelatin silver halide emulsions can be prepared using silver halide dispersing agents, e. g. starch acetate, gum arabic, a copolymer of maleic anhydride and vinyl acetate, low viscosity methyl cellulose, water-soluble amino carbohydrate dispersing agents (e. g. diethanolamine cellulose acetate or any other of these agents described in United States Patent 2,360,238, dated October 10, 1944), amino resin dispersing agents (e. g. dimethylaminobenzaldehyde acetals of polyvinyl alcohol, or water-soluble polyvinyl acetals in which at least a part of the acetal groups are 4-formylphenyltrialkylammonium salt acetal groups, such as the polyvinyl acetal of 4-formylphenyl trimethylammonium methylsulfate and other such compounds described in United States Patent 2,358,836, dated September 26, 1944), etc.

Polyvinyl compound silver halide emulsions and their preparation are described in United States Patents 2,286,216, dated June 16, 1942; 2,276,322, dated March 17, 1942; 2,276,323, dated March 17, 1942; 2,311,058, dated February 16, 1943; 2,311,059, dated February 16, 1943; 2,367,511, dated January 16, 1945; 2,376,371, dated May 22, 1945 and 2,110,491, dated March 8, 1938.

Non-gelatin proteins can also be employed as vehicles or carriers in preparing the silver halide emulsions which are stabilized in accordance with my invention. Proteins, such as casein, soybean protein, blood albumin, egg albumin, castor bean protein, globulin and edestin are examples of such non-gelatin proteins. Non gelatin proteins which have been converted to a derivative thereof, e. g. by reaction with a sulfonyl chloride, a carboxylic chloride, a carboxylic anhydride, an isocyanate, a 1,4-diketone or acrylonitrile, and then oxidized, e. g. with hydrogen peroxide, can also be employed.

My invention is directed especially to the stabilization of photographic silver halide emulsions which have been sensitized by digestion in the presence of at least one gold compound (water-soluble or water-insoluble) and in which the silver halide is principally silver bromide, but can be employed with any silver halide emulsion which has been so sensitized, particularly with the customary silver chloride, silver chlorobromide, silver chlorobromoiodide, silver chloroiodide, silver bromide and silver bromoiodide de-

veloping-out emulsions which have been so sensitized. By the term "photographic silver halide emulsion in which the silver halide is principally silver bromide," I mean a photographic silver halide emulsion in which from 60 to 100% of the weight of the silver halide is silver bromide.

Eastman Kodak Company's "D-19" developer has the following composition:

|                                |        |       |
|--------------------------------|--------|-------|
| Water                          | liters | 2.0   |
| N-methyl-p-aminophenol sulfate | grams  | 8.8   |
| Sodium sulfite, desiccated     | do     | 384.0 |
| Hydroquinone                   | do     | 35.2  |
| Sodium carbonate, desiccated   | do     | 192.0 |
| Potassium bromide              | do     | 20.0  |
| Water to make                  | liters | 4.0   |

What I claim as my invention and desire to be secured by Letters Patent of the United States is:

1. A process for stabilizing against loss of speed a photographic silver halide emulsion which has been sensitized by digesting the emulsion in the presence of a gold compound, comprising adding to the gold-compound-sensitized emulsion after the final digestion of the emulsion but prior to coating the emulsion on a support, a water-soluble gold compound which has a solubility in water greater than the equivalent of 1.0 mg. of gold per 100 ml. of water at 25° C.

2. A process for stabilizing against loss of speed a photographic gelatino-silver-halide developing-out emulsion which has been sensitized by digesting the emulsion in the presence of a gold compound, comprising adding to the gold-compound-sensitized emulsion after the final digestion of the emulsion, but prior to coating the emulsion on a support, a water-soluble gold compound which has a solubility in water greater than the equivalent of 1.0 mg. of gold per 100 ml. of water at 25° C.

3. A process for stabilizing against loss of speed a photographic gelatino-silver-halide developing-out emulsion which has been sensitized by digesting the emulsion in the presence of a gold compound, comprising adding to the gold-compound-sensitized emulsion, at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C.

4. A process for stabilizing against loss of speed a photographic gelatino-silver-halide developing-out emulsion in which the silver halide is principally silver bromide, which has been sensitized by digesting the emulsion in the presence of a gold compound, comprising adding to the gold-compound-sensitized emulsion at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

5. A process for stabilizing against loss of speed a photographic gelatino-silver-bromoiodide developing-out emulsion in which the silver halide is principally silver bromide, which has been sensitized by digesting the emulsion in the presence of a gold compound, comprising adding to the gold-compound-sensitized emulsion at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

6. A process for stabilizing against loss of speed a photographic gelatino-silver-halide developing-out emulsion in which the silver halide is principally silver bromide, which has been sensitized by digesting the emulsion in the presence of a gold compound and a sulfur sensitizing, comprising adding to the gold-compound-sensitized emulsion at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

7. A process for stabilizing against loss of speed a photographic gelatino-silver-bromoiodide developing-out emulsion in which the silver halide is principally silver bromide, which has been sensitized by digesting the emulsion in the presence of a gold compound and a sulfur sensitizing, comprising adding to the gold-compound-sensitized emulsion at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

8. A process for stabilizing against loss of speed a photographic gelatino-silver-halide developing-out emulsion in which the silver halide is principally silver bromide, which has been sensitized by digesting the emulsion in the presence of a gold compound and a thiocyanate selected from the group consisting of alkali metal and ammonium thiocyanates, comprising adding to the gold-compound-sensitized emulsion at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

9. A process for stabilizing against loss of speed a photographic gelatino-silver-bromoiodide developing-out emulsion in which the silver halide is principally silver bromide, which has been sensitized by digesting the emulsion in the presence of a gold compound and a thiocyanate selected from the group consisting of alkali metal and ammonium thiocyanates, comprising adding to the gold-compound-sensitized emulsion at a pH of from 5 to 9, after the final digestion of the emulsion, but prior to coating the emulsion on a support, a water-soluble gold compound which has a solubility in water greater than the equivalent of 1.0 mg. of gold per 100 ml. of water at 25° C., the concentration of the water-soluble gold compound being equivalent to from 1.5 to 20 mg. of gold per 1000 g. of silver nitrate used in preparing the emulsion.

10. A process for stabilizing against loss of speed a photographic gelatino-silver bromoiodide developing-out emulsion in which the silver halide is principally silver bromide, which has been sensitized by digesting the emulsion in the presence of a gold compound and a thiocyanate selected from the group consisting of alkali metal and ammonium thiocyanates, comprising adding to the gold-compound-sensitized emulsion at a pH of from 5 to 9, after the final digestion of the emulsion, but prior to coating the emulsion on a support, potassium chloroaurate in a concentration of from 1.5 to 20 mg. of gold per 1000 g. of silver nitrate used in preparing the emulsion.

11. A process for stabilizing against loss of speed a photographic gelatino-silver-bromoiodide developing-out emulsion in which the silver halide is principally silver bromide, which has been sensitized by digesting the emulsion in the presence of a gold compound and a thiocyanate selected from the group consisting of alkali metal and ammonium thiocyanates, comprising adding to the gold-compound-sensitized emulsion at a pH of from 5 to 9, after the final digestion of the emulsion, but prior to coating the emulsion on a support, potassium aurithiocyanate in a concentration of from 1.5 to 20 mg. of gold per 1000 g. of silver nitrate used in preparing the emulsion.

12. A process for stabilizing against loss of speed a photographic gelatino-silver-bromoiodide developing-out emulsion in which the silver halide is principally silver bromide, which has been sensitized by digesting the emulsion in the presence of a gold compound and a thiocyanate selected from the group consisting of alkali metal and ammonium thiocyanates, comprising adding to the gold-compound-sensitized emulsion at a pH of from 5 to 9, after the final digestion of the emulsion, but prior to coating the emulsion on a support, a water-soluble gold compound having the following formula:



in a concentration of from 1.5 to 20 mg. of gold per 1000 g. of silver nitrate used in preparing the emulsion.

13. A process for stabilizing against loss of speed a photographic gelatino-silver-bromoiodide developing-out emulsion in which the silver halide is principally silver bromide, which has been sensitized by digesting the emulsion in the presence of potassium chloroaurate, thiosinamine and sodium thiocyanate, comprising adding to the potassium-chloroaurate-sensitized emulsion at a pH of 5 to 9, after the final digestion of the emulsion, but prior to coating the emulsion on a support,

potassium chloroaurate in a concentration of from 1.5 to 20 mg. of gold per 1000 g. of silver nitrate used in preparing the emulsion.

14. A process for stabilizing against loss of speed a photographic gelatino-silver-bromoiodide developing-out emulsion in which the silver halide is principally silver bromide, which has been sensitized by digesting the emulsion in the presence of potassium chloroaurate, thiosinamine and sodium thiocyanate, comprising adding to the potassium-chloroaurate-sensitized emulsion at a pH of 5 to 9, after the final digestion of the emulsion, but prior to coating the emulsion on a support, potassium aurithiocyanate in a concentration of from 1.5 to 20 mg. of gold per 1000 g. of silver nitrate used in preparing the emulsion.

15. A process for stabilizing against loss of speed a photographic gelatino-silver bromoiodide developing-out emulsion in which the silver halide is principally silver bromide, which has been sensitized by digesting the emulsion in the presence of potassium chloroaurate, thiosinamine and sodium thiocyanate, comprising adding to the potassium-chloroaurate-sensitized emulsion at a pH of 5 to 9, after the final digestion of the emulsion, but prior to coating the emulsion on a support, a water-soluble gold compound having the following formula:



in a concentration of from 1.5 to 20 mg. of gold per 1000 g. of silver nitrate used in preparing the emulsion.

16. The emulsion obtained by the process of claim 1.

17. The emulsion obtained by the process of claim 3.

18. The emulsion obtained by the process of claim 4.

19. The emulsion obtained by the process of claim 6.

20. The emulsion obtained by the process of claim 12.

RUDOLPH E. DAMSCHRODER.

#### REFERENCES CITED

The following references are of record in the file of this patent:

#### UNITED STATES PATENTS

55 Number Name Date  
2,399,083 Waller et al. Apr. 23, 1946

#### FOREIGN PATENTS

60 Number Country Date  
608,667 Great Britain Sept. 20, 1948